# EUROPEAN PATENT APPLICATION

(11) **EP 4 782 107 A1**
(43) Date of publication of application: **29.07.2026**
(21) Application number: 25197874.8
(22) Date of filing: 25.08.2025
(51) Int. Cl.: B03D 1/004, B03D 1/008, B03D 1/01, B03D 1/016, B03D 1/018, B03D 1/08, B03C 1/30

(54) **BENEFICIATION METHODS FOR MIXED RARE EARTH ORE**

(30) Priority: 26.01.2025 CN 202510121082
(71) Applicant: Baotou Research Institute of Rare Earths, Baotou, Inner Mongolia 014030 (CN)
(72) Inventor: WANG, Weiwei, Baotou, 014030 (CN); GUO, Chunlei, Baotou, 014030 (CN); HOU, Shaochun, Baotou, 014030 (CN); LI, Qiang, Baotou, 014030 (CN); QIN, Yufang, Baotou, 014030 (CN); LI, Erdou, Baotou, 014030 (CN)
(74) Representative: Gong, Jinping

(57) **Abstract**

The present disclosure provides a beneficiation method for mixed rare earth ore, comprising: subjecting ground mixed rare earth ore to magnetic separation to produce a magnetic concentrate and a magnetic tailing, wherein the mixed rare earth ore contains carbocernaite and parisite; subjecting the magnetic concentrate to first flotation in the presence of a pH regulator A, a depressant A, a collector A, and a frother A to produce a first flotation concentrate and a first flotation tailing, wherein the depressant A comprises water glass, a phosphate, and starch, the collector A comprises a hydroxamic acid and a styrylphenol polyoxyethylene ether, and the frother A is a fatty alcohol frother; grinding the first flotation tailing to produce a ground first flotation tailing; and subjecting the ground first flotation tailing to second flotation in the presence of a pH regulator B, a depressant B, a collector B, and a frother B to produce a second flotation concentrate. The beneficiation method of the present disclosure can increase the rare earth grade of mixed rare earth ore containing carbocernaite and parisite.

## Description

### TECHNICAL FIELD OF THE DISCLOSURE

The present disclosure relates to a beneficiation method for mixed rare earth ore.

### BACKGROUND OF THE DISCLOSURE

Rare earth elements include lanthanides, yttrium, and scandium. These elements possess unique spatial structures and physicochemical properties, making them indispensable in various high-tech fields. Known as the "vitamins of industry," rare earth elements serve as fundamental raw materials for many critical and advanced technological applications. In nature, rare earth elements typically occur in the form of bastnaesite, monazite, and xenotime. Carbocernaite [(Ce,Na,Sr,Ca)CO₃] is often found in carbonate rocks and alkaline rocks, particularly in regions associated with hydrothermal activity, and it is often found alongside other rare earth minerals such as parisite, bastnaesite, and apatite. Current research on the enrichment of rare earth element resources primarily focuses on bastnaesite, monazite, and xenotime, with relatively few studies dedicated to carbocernaite.

CN103962232A discloses a beneficiation method for rare earth ore, which comprises: grinding raw ore into particles 100% of which have a particle size of 2.00 mm or less, and classifying the particles into three size fractions of -2.00 +0.65 mm fraction, -0.65 +0.074 mm fraction, and -0.074 mm fraction; subjecting the -2.00 +0.65 mm fraction to gravity separation using a spiral concentrator to produce a spiral concentrate and a spiral tailing; subjecting the -0.65 +0.074 mm fraction to spiral chute gravity separation to produce a spiral chute concentrate and a spiral chute tailing; subjecting the -0.074 mm fraction to magnetic separation at a field intensity of 1.0-1.5 T to produce a high-intensity magnetic concentrate and a high-intensity magnetic tailing; subjecting the spiral concentrate, the spiral chute concentrate, and the high-intensity magnetic concentrate to shaking table separation separately to produce a table concentrate, a table middling, and a table tailing; combining the table concentrate and the table middling from all the fractions and subjecting them to wet high-gradient magnetic separation at a field intensity of 0.4-0.9 T to produce a magnetic rare earth concentrate and a magnetic middling; combining the magnetic middling and the table tailing and regrinding them into a slurry that comprises particles 50-85% of which have a particle size of 0.043 mm or less and that has a concentration of 20-45%, conditioning the slurry with a regulator in an amount of 1000-3000 g per ton of the raw ore, subjecting the conditioned slurry to rougher flotation with a collector in an amount of 1000-2500 g per ton of the raw ore and with kerosene as the frother in an amount of 30-80 g per ton of the raw ore to produce a rougher flotation concentrate and a rougher flotation tailing; subjecting a slurry of the rougher flotation tailing (having a concentration of 20-35%) to first scavenger flotation with a collector in an amount of 1000-1500 g per ton of the raw ore and with kerosene as the frother in an amount of 5-40 g per ton of the raw ore to produce a first scavenger flotation concentrate (returned to the rougher flotation) and a first scavenger flotation tailing; subjecting a slurry of the first scavenger flotation tailing (having a concentration of 20-35%) to second scavenger flotation with a collector in an amount of 400-800 g per ton of the raw ore to produce a second scavenger flotation concentrate (returned to the first scavenger flotation) and a second scavenger flotation tailing; subjecting a slurry of the rougher flotation concentrate (having a concentration of 10-20%) to first cleaner flotation with a regulator in an amount of 400-800 g per ton of the raw ore to produce a first cleaner flotation concentrate and a first cleaner flotation tailing (returned to the rougher flotation); subjecting a slurry of the first cleaner flotation concentrate (having a concentration of 3-15%) to second cleaner flotation with a regulator in an amount of 200-600 g per ton of the raw ore to produce a flotation rare earth concentrate and a second cleaner flotation tailing (returned to the first cleaner flotation); and combining the magnetic rare earth concentrate and the flotation rare earth concentrate to produce a total rare earth concentrate. This method is particularly applicable to mixed rare earth ore containing bastnaesite, parisite, and monazite.

CN102500465A discloses a beneficiation method for bastnaesite, comprising: grinding raw ore into particles having a particle size of 1.0 mm or less, and classifying the particles into three size fractions of -1.0 +0.4 mm fraction, -0.4 +0.074 mm fraction, and -0.074 mm fraction; subjecting each of the three fractions to magnetic separation at a field intensity of 1.0 T to produce a high-intensity magnetic concentrate and a high-intensity magnetic tailing; subjecting each of the high-intensity magnetic concentrates to shaking table separation to produce a table concentrate, a table middling, and a table tailing; combining the table concentrates and the table middling from all the fractions and subjecting them to wet high-gradient magnetic separation at a rated background field intensity of 0.5-0.8 T to produce a magnetic bastnaesite concentrate and a magnetic middling; combining the magnetic middling and the table tailing and regrinding them into a slurry that comprises particles 50-75% of which have a particle size of 0.043 mm or less and that has a concentration of 25-35%, conditioning the slurry with a regulator in an amount of 1000-3000 g per ton of the raw ore, and subjecting the conditioned slurry to rougher flotation with a collector in an amount of 3000-5000 g per ton of the raw ore and with No. 2 oil as the frother in an amount of 10-100 g per ton of the raw ore to produce a rougher flotation concentrate and a rougher flotation tailing; subjecting a slurry of the rougher flotation tailing (having a concentration of 20-30%) to first scavenger flotation with a collector in an amount of 1000-1500 g per ton of the raw ore and with No. 2 oil as the frother in an amount of 5-40 g per ton of the raw ore to produce a first scavenger flotation concentrate (returned to the rougher flotation) and a first scavenger flotation tailing; subjecting a slurry of the first scavenger flotation tailing (having a concentration of 20-35%) to second scavenger flotation with a collector in an amount of 400-800 g per ton of the raw ore to produce a second scavenger flotation concentrate (returned to the second scavenger flotation) and a second scavenger flotation tailing; subjecting a slurry of the rougher flotation concentrate (having a concentration of 10-30%) to first cleaner flotation with a regulator in an amount of 400-1000 g per ton of the raw ore to produce a first cleaner flotation concentrate and a first cleaner flotation tailing (returned to the rougher flotation); subjecting a slurry of the first cleaner flotation concentrate (having a concentration of 10-25%) to second cleaner flotation with a regulator in an amount of 200-800 g per ton of the raw ore to produce a second cleaner flotation concentrate and a second cleaner flotation tailing (returned to the first cleaner flotation); and subjecting a slurry of the second cleaner flotation concentrate (having a concentration of 5-20%) to third cleaner flotation with a regulator in an amount of 100-400 g per ton of the raw ore to produce a flotation bastnaesite concentrate and a third cleaner flotation tailing (returned to the second cleaner flotation). This method is applicable to bastnaesite.

### SUMMARY OF THE DISCLOSURE

One objective of the present disclosure is to provide a beneficiation method for mixed rare earth ore. The beneficiation method of the present disclosure can effectively increase the rare earth grade of mixed rare earth ore containing carbocernaite and parisite. Also, the beneficiation method achieves a high rare earth recovery rate. The objective of the present disclosure is accomplished by technical solutions described below.

The present disclosure provides a beneficiation method for mixed rare earth ore, comprising:
(1) subjecting ground mixed rare earth ore to magnetic separation to produce a magnetic concentrate and a magnetic tailing, wherein the mixed rare earth ore contains carbocernaite and parisite;
(2) subjecting the magnetic concentrate to first flotation in the presence of a pH regulator A, a depressant A, a collector A, and a frother A to produce a first flotation concentrate and a first flotation tailing,
   wherein the depressant A comprises water glass, a phosphate, and starch in a mass ratio of (4-8):(1-5):(0.5-3), the collector A comprises a C5-C10 hydroxamic acid and a styrylphenol polyoxyethylene ether in a mass ratio of (7-11):(0.5-3), and the frother A is a fatty alcohol frother;
(3) grinding the first flotation tailing to produce a ground first flotation tailing; and
(4) subjecting the ground first flotation tailing to second flotation in the presence of a pH regulator B, a depressant B, a collector B, and a frother B to produce a second flotation concentrate and a second flotation tailing,
   wherein the depressant B comprises water glass, a phosphate, and starch in a mass ratio of (4-8):(1-5):(0.5-3), the collector B comprises a C5-C10 hydroxamic acid and a styrylphenol polyoxyethylene ether in a mass ratio of (7-11):(0.5-3), and the frother B is a fatty alcohol frother.

In the beneficiation method according to the present disclosure, preferably, step (1) comprises:
subjecting ground mixed rare earth ore to rougher magnetic separation to produce a rougher magnetic concentrate and a rougher magnetic tailing, wherein the rougher magnetic separation is performed at a field intensity of 1.1-1.5 T and a pulse frequency of 12-16 Hz and uses the ground mixed rare earth ore having a concentration of 10-30 wt%;
subjecting the rougher magnetic tailing to scavenger magnetic separation to produce a scavenger magnetic concentrate and a magnetic tailing, wherein the scavenger magnetic separation is performed at a field intensity of 1.6-2.0 T and a pulse frequency of 13-20 Hz and uses the rougher magnetic tailing having a concentration of 10-30 wt%; and
combining the rougher magnetic concentrate and the scavenger magnetic concentrate to produce a magnetic concentrate,
wherein the ground mixed rare earth ore consists of particles 75-100 wt% of which have a particle size of 0.074 mm or less.

In the beneficiation method according to the present disclosure, preferably, the water glass has a modulus of 2-3, the phosphate is one or more selected from the group consisting of sodium hexametaphosphate and trisodium phosphate, the hydroxamic acid is a C7-9 hydroxamic acid, the styrylphenol polyoxyethylene ether is one or more selected from the group consisting of pesticide emulsifier 601, pesticide emulsifier 602, pesticide emulsifier 603, and pesticide emulsifier 604, the fatty alcohol frother is a C4-C10 aliphatic monohydric alcohol, the pH regulator A is a carbonate, and the pH regulator B is a carbonate.

In the beneficiation method according to the present disclosure, preferably, step (2) comprises:
forming a magnetic concentrate slurry having a concentration of 45-65 wt% from the magnetic concentrate; subjecting the magnetic concentrate slurry to first rougher flotation by adding thereto at 50-70 °C a pH regulator A, a depressant A, a collector A, and a frother A to produce a first rougher flotation concentrate and a first flotation tailing, wherein the pH regulator A is in an amount of 1.0-2.0 kg/T, the depressant A is in an amount of 1.5-2.5 kg/T, the collector A is in an amount of 0.9-1.5 kg/T, and the frother A is in an amount of 0.1-0.3 kg/T, based on the weight of the mixed rare earth ore; and
subjecting the first rougher flotation concentrate to N-stage first cleaner flotation to produce a first flotation concentrate, wherein N is an integer greater than or equal to 2,
wherein 1^{st}-stage first cleaner flotation comprises: forming a first rougher flotation concentrate slurry from the first rougher flotation concentrate; subjecting the first rougher flotation concentrate slurry to 1^{st}-stage first cleaner flotation by adding thereto a pH regulator A, a depressant A, a collector A, and a frother A to produce a 1^{st}-stage first cleaner flotation concentrate and a 1^{st}-stage first cleaner flotation tailing; and returning the 1^{st}-stage first cleaner flotation tailing as a feed material to the first rougher flotation, wherein the pH regulator A is in an amount of 0.2-0.6 kg/T, the depressant A is in an amount of 0.4-0.9 kg/T, the collector A is in an amount of 0.1-0.5 kg/T, and the frother A is in an amount of 0.01-0.2 kg/T, based on the weight of the mixed rare earth ore, and
wherein each of 2^{nd}-stage first cleaner flotation to N^{th}-stage first cleaner flotation comprises:
   forming a (m-1)^{th}-stage first cleaner flotation concentrate slurry from a (m-1)^{th}-stage first cleaner flotation concentrate; subjecting the (m-1)^{th}-stage first cleaner flotation concentrate slurry to m^{th}-stage first cleaner flotation by adding thereto a pH regulator A, a depressant A, a collector A, and a frother A to produce a m^{th}-stage first cleaner flotation concentrate and a m^{th}-stage first cleaner flotation tailing; and returning the m^{th}-stage first cleaner flotation tailing as a feed material to the (m-1)^{th}-stage first cleaner flotation, wherein the pH regulator A is in an amount of 0.05-0.25 kg/T, the depressant A is in an amount of 0.10-0.35 kg/T, the collector A is in an amount of 0.05-0.25 kg/T, and the frother A is in an amount of 0.005-0.035 kg/T, based on the weight of the mixed rare earth ore, m is an integer greater than or equal to 2 and less than or equal to N, and the N^{th}-stage first cleaner flotation concentrate is the first flotation concentrate.

In the beneficiation method according to the present disclosure, preferably in step (2), the pH regulator A, the depressant A, the collector A, and the frother A are added in this order at an interval of 2-5 minutes,
wherein the interval is calculated by the following formula: $t = {t}_{1} - {t}_{2}$ where t is the interval, t₁ is the time of starting the addition of a next reagent, and t₂ is the time of completing the addition of a preceding reagent.

In the beneficiation method according to the present disclosure, preferably in step (3), the first flotation tailing for grinding has a concentration of 50-65 wt%, and the ground first flotation tailing consists of particles 85-100 wt% of which have a particle size of 0.03 mm or less.

In the beneficiation method according to the present disclosure, preferably step (4) comprises:
forming a first flotation tailing slurry having a concentration of 40-65 wt% from the ground first flotation tailing; subjecting the first flotation tailing slurry to second rougher flotation by adding thereto at 50-70 °C a pH regulator B, a depressant B, a collector B, and a frother B to produce a second rougher flotation concentrate and a second flotation tailing, wherein the pH regulator B is in an amount of 0.6-1.3 kg/T, the depressant B is in an amount of 0.8-1.6 kg/T, the collector B is in an amount of 0.5-1.1 kg/T, and the frother B is in an amount of 0.1-0.5 kg/T, based on the weight of the mixed rare earth ore; and
subjecting the second rougher flotation concentrate to I-stage second cleaner flotation to produce a second flotation concentrate, wherein I is an integer greater than or equal to 2,
wherein 1^{st}-stage second cleaner flotation comprises:
   forming a second rougher flotation concentrate slurry from the second rougher flotation concentrate; subjecting the second rougher flotation concentrate slurry to 1^{st}-stage second cleaner flotation by adding thereto a pH regulator B, a depressant B, a collector B, and a frother B to produce a 1^{st}-stage second cleaner flotation concentrate and a 1^{st}-stage second cleaner flotation tailing; and returning the 1^{st}-stage second cleaner flotation tailing as a feed material to the second rougher flotation, wherein the pH regulator B is in an amount of 0.2-0.5 kg/T, the depressant B is in an amount of 0.2-0.6 kg/T, the collector B is in an amount of 0.1-0.5 kg/T, and the frother B is in an amount of 0.01-0.15 kg/T, based on the weight of the mixed rare earth ore,
   wherein each of 2^{nd}-stage second cleaner flotation to I^{th}-stage second cleaner flotation comprises:
      forming a (j-1)^{th}-stage second cleaner flotation concentrate slurry from a (j-1)^{th}- stage second cleaner flotation concentrate; subjecting the (j-1)^{th}-stage second cleaner flotation concentrate slurry to j^{th}-stage second cleaner flotation by adding thereto a pH regulator B, a depressant B, a collector B, and a frother B to produce a j^{th}-stage second cleaner flotation concentrate and a j^{th}-stage second cleaner flotation tailing; and returning the j^{th}-stage second cleaner flotation tailing as a feed material to the (j-1)^{th}-stage second cleaner flotation, wherein the pH regulator B is in an amount of 0.05-0.30 kg/T, the depressant B is in an amount of 0.08-0.35 kg/T, the collector B is in an amount of 0.05-0.25 kg/T, and the frother B is in an amount of 0.005-0.07 kg/T, based on the weight of the mixed rare earth ore, j is an integer greater than or equal to 2 and less than or equal to I, and the I^{th}-stage second cleaner flotation concentrate is the second flotation concentrate.

In the beneficiation method according to the present disclosure, preferably in step (4), the pH regulator B, the depressant B, the collector B, and the frother B are added in this order at an interval of 2-5 minutes,
wherein the interval is calculated by the following formula: $t = {t}_{1} - {t}_{2}$ where t is the interval, t₁ is the time of starting the addition of a next reagent, and t₂ is the time of completing the addition of a preceding reagent.

the beneficiation method according to the present disclosure preferably comprises:
combining the first flotation concentrate and the second flotation concentrate to produce a rare earth concentrate.

The beneficiation method according to the present disclosure preferably further comprises:
crushing the mixed rare earth ore to produce crushed ore; and grinding the crushed ore to produce ground mixed rare earth ore,
wherein the mixed rare earth ore contains carbocernaite and parisite in a mass ration of (3-6.5):(2-5.5), and further contains at least one of calcite, mica, feldspar, and apatite.

The beneficiation method of the present disclosure enables the enrichment of carbocernaite and parisite from mixed rare earth ore, thereby making a rare earth concentrate containing high-grade rare earth available. Also, the beneficiation method of the present disclosure achieves a high rare earth recovery rate.

### DETAIL DESCRIPTION OF THE DISCLOSURE

The following is a further description of the present disclosure by means of embodiments, but the present disclosure is not limited to those embodiments.

The beneficiation method for mixed rare earth ore of the present disclosure comprises: (1) magnetic separation; (2) first flotation; (3) grinding of first flotation tailing; and (4) second flotation. In some embodiments, the method further comprises crushing and grinding the mixed rare earth ore. Each of these steps is hereinafter described in detail.

### Magnetic Separation

The present disclosure involves subjecting ground mixed rare earth ore to magnetic separation to produce a magnetic concentrate and a magnetic tailing.

The mixed rare earth ore of the present disclosure contains carbocernaite and parisite. The mass ratio of carbocernaite to parisite is (3-6.5):(2-5.5), preferably (4-6):(3-5). In some embodiments, the mass ratio of carbocernaite to parisite is (4.5-5):(3.5-4).

The rare earth grade of the mixed rare earth ore may be 2.5-5.5 wt%, preferably 3-4.5 wt%. In certain embodiments, the rare earth grade of the mixed rare earth ore is 3.5-3.8 wt%.

The mixed rare earth ore further contains a gangue selected from at least one of calcite, mica, feldspar, and apatite. Calcite may be contained in the mixed rare earth ore in an amount of 35-55 wt%, preferably 40-50 wt%, and more preferably 42-46 wt%.

The ground mixed rare earth ore consists of particles 75-100 wt% of which, preferably 80-95 wt% of which, and more preferably 85-90 wt% of which have a particle size of 0.074 mm or less.

In the ground mixed rare earth ore, carbocernaite may have a liberation degree of 75-90 wt%. In some embodiments, carbocernaite has a liberation degree of 80-87 wt%.

In the ground mixed rare earth ore, parisite may have a liberation degree of 20-35 wt%. In some embodiments, parisite has a liberation degree of 24-30 wt%.

Specifically, the magnetic separation comprises: subjecting ground mixed rare earth ore to rougher magnetic separation to produce a rougher magnetic concentrate and a rougher magnetic tailing; subjecting the rougher magnetic tailing to scavenger magnetic separation to produce a scavenger magnetic concentrate and a magnetic tailing; and combining the rougher magnetic concentrate and the scavenger magnetic concentrate to produce a magnetic concentrate.

The parameters in the rougher magnetic separation are as follows:
The magnetic field intensity may be 1.1-1.5 T, preferably 1.2-1.4 T, and more preferably 1.2-1.3 T.

The ground mixed rare earth ore may have a concentration of 10-30 wt%, preferably 15-25 wt%, and more preferably 20-22 wt%.

The pulse frequency may be 12-16 Hz, preferably 13-15 Hz, and more preferably 14-15 Hz.

The parameters in the scavenger magnetic separation are as follows:
The magnetic field intensity may be 1.6-2.0 T, preferably 1.7-1.9 T, and more preferably 1.7-1.8 T.

The rougher magnetic tailing may have a concentration of 10-30 wt%, preferably 15-25 wt%, and more preferably 20-22 wt%.

The pulse frequency may be 13-20 Hz, preferably 15-19 Hz, and more preferably 17-18 Hz.

### First Flotation

The present disclosure involves subjecting the magnetic concentrate to first flotation in the presence of a pH regulator A, a depressant A, a collector A, and a frother A to produce a first flotation concentrate and a first flotation tailing. The letter "A" in these reagents has no special meaning and is only used to distinguish them from reagents used in second flotation described hereinafter.

The pH regulator A may be a carbonate, preferably an alkali metal carbonate, such as sodium carbonate or potassium carbonate. In one embodiment of the present disclosure, the pH regulator A is potassium carbonate.

The depressant A comprises water glass, a phosphate, and starch. The mass ratio between water glass, the phosphate, and starch may be (4-8):(1-5):(0.5-3), preferably (5-7):(2-4):(0.8-2), and more preferably (6-6.5):(3-3.5):(1-1.5).

The modulus of water glass may be 2-3, preferably 2.2-2.8, and more preferably 2.4-2.6.

The phosphate may be selected from one or more of sodium hexametaphosphate and trisodium phosphate, and it is preferably sodium hexametaphosphate.

The collector A comprises a hydroxamic acid and a styrylphenol polyoxyethylene ether. The mass ratio of the hydroxamic acid to the styrylphenol polyoxyethylene ether may be (7-11):(0.5-3), preferably (8-10):(0.5-2), and more preferably (9-9.5):(1-1.5).

The hydroxamic acid may be a C5-C10 hydroxamic acid, preferably a C7-C9 hydroxamic acid, more preferably a C8 hydroxamic acid, and most preferably octyl hydroxamic acid (octanohydroxamic acid).

The styrylphenol polyoxyethylene ether may be selected from one or more of pesticide emulsifiers 601, 602, 603, and 604, and it is preferably pesticide emulsifier 601.

The frother A is an aliphatic alcohol frother, preferably a C4-C10 aliphatic monohydric alcohol, more preferably a C6-C8 aliphatic monohydric alcohol, and most preferably methyl isobutyl carbinol.

Specifically, the first flotation comprises: forming a magnetic concentrate slurry from the magnetic concentrate, subjecting the magnetic concentrate slurry to first rougher flotation by adding thereto a pH regulator A, a depressant A, a collector A, and a frother A to produce a first rougher flotation concentrate and a first flotation tailing, and subjecting the first rougher flotation concentrate to N-stage first cleaner flotation to produce a first flotation concentrate. N is an integer greater than or equal to 2, preferably, N is an integer between 3 and 5 inclusive, and most preferably, N is 3.

The concentration of the magnetic concentrate slurry may be 45-65 wt%, preferably 50-60 wt%, and more preferably 55-60 wt%.

The first rougher flotation may be carried out at a temperature of 50-70 °C, preferably 55-65 °C, and more preferably 60-65 °C.

In the first rougher flotation, the pH regulator A may be in an amount of 1.0-2.0 kg/T, preferably 1.2-1.8 kg/T, and more preferably 1.4-1.6 kg/T, based on the weight of the mixed rare earth ore.

In the first rougher flotation, the depressant A may be in an amount of 1.5-2.5 kg/T, preferably 1.7-2.3 kg/T, and more preferably 2-2.2 kg/T, based on the weight of the mixed rare earth ore.

In the first rougher flotation, the collector A may be in an amount of 0.9-1.5 kg/T, preferably 1-1.3 kg/T, and more preferably 1.1-1.2 kg/T, based on the weight of the mixed rare earth ore.

In the first rougher flotation, the frother A may be in an amount of 0.1-0.3 kg/T, preferably 0.15-0.25 kg/T, and more preferably 0.18-0.2 kg/T, based on the weight of the mixed rare earth ore.

In the first rougher flotation, the pH regulator A, the depressant A, the collector A, and the frother A may be added in this order to the magnetic concentrate slurry.

These reagents are added at an interval of 2-5 minutes, preferably 3-4 minutes. The interval is calculated by the following formula: t=t₁-t₂, where t is the interval, t₁ is the time of starting the addition of a next reagent, and t₂ is the time of completing the addition of a preceding reagent.

Specifically, the 1^{st}-stage first cleaner flotation comprises: forming a first rougher flotation concentrate slurry from the first rougher flotation concentrate, and subjecting the first rougher flotation concentrate slurry to 1^{st}-stage first cleaner flotation by adding a pH regulator A, a depressant A, a collector A, and a frother A to produce a 1^{st}-stage first cleaner flotation concentrate and a 1^{st}-stage first cleaner flotation tailing; and returning the 1^{st}-stage first cleaner flotation tailing as a feed material to the first rougher flotation.

In the 1^{st}-stage first cleaner flotation, the pH regulator A is in an amount of 0.2-0.6 kg/T, preferably 0.3-0.5 kg/T, and more preferably 0.4-0.45 kg/T, based on the weight of the mixed rare earth ore.

In the 1^{st}-stage first cleaner flotation, the depressant A is 0.4-0.9 kg/T, preferably 0.5-0.8 kg/T, and more preferably 0.6-0.7 kg/T, based on the weight of the mixed rare earth ore.

In the 1^{st}-stage first cleaner flotation, the collector A is in an amount of 0.1-0.5 kg/T, preferably 0.2-0.45 kg/T, and more preferably 0.3-0.4 kg/T, based on the weight of the mixed rare earth ore.

In the 1^{st}-stage first cleaner flotation, the frother A is in an amount of 0.01-0.2 kg/T, preferably 0.03-0.1 kg/T, and more preferably 0.05-0.08 kg/T, based on the weight of the mixed rare earth ore.

In the 1^{st}-stage first cleaner flotation, the pH regulator A, the depressant A, the collector A, and the frother A may be added in this order to the first rougher flotation concentrate slurry.

These reagents are added at an interval of 2-5 minutes, preferably 3-4 minutes. The interval is calculated by the following formula: t=t₁-t₂, where t is the interval, t₁ is the time of starting the addition of a next reagent, and t₂ is the time of completing the addition of a preceding reagent.

The concentration of the first rougher flotation concentrate slurry may be 40-70 wt%, preferably 45-65 wt%, and more preferably 50-60 wt%.

The 1^{st}-stage first cleaner flotation may be carried out at a temperature of 35-65 °C, preferably 40-60 °C, and more preferably 50-55 °C.

Specifically, each of 2^{nd}-stage first cleaner flotation to N^{th}-stage first cleaner flotation comprises:
forming a (m-1)^{th}-stage first cleaner flotation concentrate slurry from a (m-1)^{th}-stage first cleaner flotation concentrate; subjecting the (m-1)^{th}-stage first cleaner flotation concentrate slurry to m^{th}-stage first cleaner flotation by adding thereto a pH regulator A, a depressant A, a collector A, and a frother A to produce a m^{th}-stage first cleaner flotation concentrate and a m^{th}-stage first cleaner flotation tailing; and returning the m^{th}-stage first cleaner flotation tailing as a feed material to the (m-1)^{th}-stage first cleaner flotation. In the present disclosure, m is an integer greater than or equal to 2 and less than or equal to N, and the N^{th}-stage first cleaner flotation concentrate is the first flotation concentrate.

In the m^{th}-stage first cleaner flotation, the pH regulator A may be in an amount of 0.05-0.25 kg/T, preferably 0.10-0.20 kg/T, and more preferably 0.12-0.16 kg/T, based on the weight of the mixed rare earth ore.

In the m^{th}-stage first cleaner flotation, the depressant A may be in an amount of 0.10-0.35 kg/T, preferably 0.15-0.30 kg/T, and more preferably 0.20-0.25 kg/T, based on the weight of the mixed rare earth ore.

In the m^{th}-stage first cleaner flotation, the collector A may be in an amount of 0.05-0.25 kg/T, preferably 0.10-0.20 kg/T, and more preferably 0.12-0.15 kg/T, based on the weight of the mixed rare earth ore.

In the m^{th}-stage first cleaner flotation, the frother A may be in an amount of 0.005-0.035 kg/T, preferably 0.010-0.030 kg/T, and more preferably 0.015-0.020 kg/T, based on the weight of the mixed rare earth ore.

In the m^{th}-stage first cleaner flotation, the pH regulator A, the depressant A, the collector A, and the frother A may be added in this order to the (m-1)^{th}-stage first cleaner flotation concentrate slurry.

These reagents are added at an interval of 2-5 minutes, preferably 3-4 minutes. The interval is calculated by the following formula: t=t₁-t₂, where t is the interval, t₁ is the time of starting the addition of a next reagent, and t₂ is the time of completing the addition of a preceding reagent.

The concentration of the (m-1)^{th}-stage first cleaner flotation concentrate slurry may be 35-65 wt%, preferably 40-60 wt%, and more preferably 45-50 wt%.

The m^{th}-stage first cleaner flotation may be carried out at a temperature of 35-65 °C, preferably 45-60 °C, and more preferably 50-55 °C.

Preferably, N is 3, meaning that three-stage first cleaner flotation is carried out.

### Grinding of First Flotation Tailing

The present disclosure involves grinding the first flotation tailing to produce a ground first flotation tailing.

The ground first flotation tailing consists of particles, 85-100 wt% of which, preferably 90-97 wt% of which have a particle size of 0.03 mm or less.

The first flotation tailing for grinding may have a concentration of 50-65 wt%, preferably 55-60 wt%.

In the ground first flotation tailing, parisite has a liberation degree of 70-90 wt%, preferably 75-85 wt%.

### Second Flotation

The present invention involves subjecting the ground first flotation tailing to second flotation in the presence of a pH regulator B, a depressant B, a collector B, and a frother B to produce a second flotation concentrate and a second flotation tailing. The reagents A and the reagents B may be identical with each other or different from each other. When the reagents A and the reagents B are identical with each other, the appended letters may be omitted. For example, when the pH regulator A and the pH regulator B are identical with each other, they may be collectively referred to as the pH regulator.

The pH regulator B may be a carbonate, preferably an alkali metal carbonate, such as sodium carbonate or potassium carbonate. In one embodiment of the present disclosure, the pH regulator B is potassium carbonate.

The depressant B comprises water glass, a phosphate, and starch. The mass ratio between water glass, the phosphate, and starch may be (4-8):(1-5):(0.5-3), preferably (5-7):(2-4):(0.8-2), and more preferably (6-6.5):(3-3.5):(1-1.5).

The modulus of water glass may be 2-3.5, preferably 2.2-2.8, and more preferably 2.4-2.6.

The phosphate may be selected from one or more of sodium hexametaphosphate and trisodium phosphate, and it is preferably sodium hexametaphosphate.

The collector B comprises hydroxamic acid and styrylphenol polyoxyethylene ether. The mass ratio of hydroxamic acid to styrylphenol polyoxyethylene ether may be (7-11):(0.5-3), preferably (8-10):(0.5-2), and more preferably (9-9.5):(1-1.5).

The hydroxamic acid may a C5-C10 hydroxamic acid, preferably a C7-C9 hydroxamic acid, more preferably a C8 hydroxamic acid, and most preferably octyl hydroxamic acid.

The styrylphenol polyoxyethylene ether may be selected from one or more of pesticide emulsifiers 601, 602, 603, and 604, and it is preferably pesticide emulsifier 601.

The frother B is an aliphatic alcohol frother, preferably a C4-C10 aliphatic monohydric alcohol, more preferably a C6-C8 aliphatic monohydric alcohol, and most preferably methyl isobutyl carbinol.

Specifically, the second flotation comprises: forming a first flotation tailing slurry from the ground first flotation tailing; subjecting the first flotation tailing slurry to second rougher flotation by adding thereto a pH regulator B, a depressant B, a collector B, and a frother B to produce a second rougher flotation concentrate and a second flotation tailing; and subjecting the second rougher flotation concentrate to I-stage second cleaner flotation to produce a second flotation concentrate. I is an integer greater than or equal to 2, preferably I is an integer between 3 and 5 inclusive; and most preferably I is 3.

The first flotation tailing slurry may have a concentration of 40-65 wt%, preferably 45-60 wt%. In some embodiments, the first flotation tailing slurry has a concentration of 50-55 wt%.

The second rougher flotation may be carried out at a temperature of 50-70 °C, preferably 55-65 °C, and more preferably 60-65 °C.

In the second rougher flotation, the pH regulator B may be in an amount of 0.6-1.3 kg/T, preferably 0.8-1.1 kg/T, based on the weight of the mixed rare earth ore. In some embodiments, the pH regulator B is in an amount of 0.8-0.9 kg/T.

In the second rougher flotation, the depressant B may be in an amount of 0.8-1.6 kg/T, preferably 1.0-1.3 kg/T, based on the weight of the mixed rare earth ore. In some embodiments, the depressant B is in an amount of 1.1-1.2 kg/T.

In the second rougher flotation, the collector B may be in an amount of 0.5-1.1 kg/T, preferably 0.7-1 kg/T, and more preferably 0.75-0.9 kg/T, based on the weight of the mixed rare earth ore.

In the second rougher flotation, the frother B may be in an amount of 0.1-0.5 kg/T, preferably 0.15-0.3 kg/T, and more preferably 0.2-0.25 kg/T, based on the weight of the mixed rare earth ore.

In the second rougher flotation, the pH regulator B, the depressant B, the collector B, and the frother B may be added in this order to the ground first flotation tailing slurry.

These reagents are added at an interval of 2-5 minutes, preferably 3-4 minutes. The interval is calculated by the following formula: t=t₁-t₂, where t is the interval, t₁ is the time of starting the addition of a next reagent, and t₂ is the time of completing the addition of a preceding reagent.

Specifically, 1^{st}-stage second cleaner flotation comprises: forming a second rougher flotation concentrate slurry from the second rougher flotation concentrate; subjecting the second rougher flotation concentrate slurry to 1^{st}-stage second cleaner flotation by adding thereto a pH regulator B, a depressant B, a collector B, and a frother B to produce a 1^{st}-stage second cleaner flotation concentrate and a 1^{st}-stage second cleaner flotation tailing; and returning the 1^{st}-stage second cleaner flotation tailing as a feed material to the second rougher flotation.

In the 1^{st}-stage second cleaner flotation, the pH regulator B may be in an amount of 0.2-0.5 kg/T, preferably 0.3-0.4 kg/T, and more preferably 0.3-0.35 kg/T, based on the weight of the mixed rare earth ore.

In the 1^{st}-stage second cleaner flotation, the depressant B is an an amount of 0.2-0.6 kg/T, preferably 0.3-0.5 kg/T, and more preferably 0.35-0.45 kg/T, based on the weight of the mixed rare earth ore.

In the 1^{st}-stage second cleaner flotation, the collector B is in an amount of 0.1-0.5 kg/T, preferably 0.2-0.4 kg/T, based on the weight of the mixed rare earth ore. In some embodiments, the collector B is in an amount of 0.3-0.35 kg/T.

In the 1^{st}-stage second cleaner flotation, the frother B is in an amount of 0.01-0.15 kg/T, preferably 0.05-0.10 kg/T, and more preferably 0.07-0.08 kg/T, based on the weight of the mixed rare earth ore.

In the 1^{st}-stage second cleaner flotation, the pH regulator B, the depressant B, the collector B, and the frother B are added in this order to the second rougher flotation concentrate slurry.

These reagents are added at an interval of 2-5 minutes, preferably 3-4 minutes. The interval is calculated by the following formula: t=t₁-t₂, where t is the interval, t₁ is the time of starting the addition of a next reagent, and t₂ is the time of completing the addition of a preceding reagent.

The concentration of the second rougher flotation concentrate slurry may be 35-60 wt%, preferably 40-55 wt%, and more preferably 45-50 wt%.

The 1^{st}-stage second cleaner flotation is carried out at a temperature of 35-65 °C, preferably 40-60 °C, and more preferably 50-55 °C.

Specifically, each of 2^{nd}-stage second cleaner flotation to I^{th}-stage second cleaner flotation comprises:
forming a (j-1)^{th}-stage second cleaner flotation concentrate slurry from a (j-1)^{th}-stage second cleaner flotation concentrate; subjecting the (j-1)^{th}-stage second cleaner flotation concentrate slurry to j^{th}-stage second cleaner flotation by adding thereto a pH regulator B, a depressant B, a collector B, and a frother B to produce a j^{th}-stage second cleaner flotation concentrate and a j^{th}-stage second cleaner flotation tailing; and returning the j^{th}-stage second cleaner flotation tailing as a feed material to the (j-1)^{th}-stage second cleaner flotation. In the present disclosure, j is an integer greater than or equal to 2 and less than or equal to I, and the I^{th}-stage second cleaner flotation concentrate is the second flotation concentrate.

In the j^{th}-stage second cleaner flotation, the pH regulator B is in an amount of 0.05-0.30 kg/T, preferably 0.08 to 0.25 kg/T, based on the weight of the mixed rare earth ore. In some embodiments, the pH regulator B is in an amount of 0.20 to 0.23 kg/T.

In the j^{th}-stage second cleaner flotation, the depressant B is in an amount of 0.08 to 0.35 kg/T, preferably 0.10 to 0.30 kg/T, based on the weight of the mixed rare earth ore. In some embodiments, the depressant B is in an amount of 0.25 to 0.28 kg/T.

In the j^{th}-stage second cleaner flotation, the collector B is in an amount of 0.05 to 0.25 kg/T, preferably 0.08 to 0.20 kg/T, based on the weight of the mixed rare earth ore. In some embodiments, the collector B is in an amount of 0.15 to 0.18 kg/T.

In the j^{th}-stage second cleaner flotation, the frother B is in an amount of 0.005 to 0.07 kg/T, preferably 0.02 to 0.06 kg/T, based on the weight of the mixed rare earth ore. In some embodiments, the frother B is in an amount of 0.045 to 0.05 kg/T.

In the j^{th}-stage second cleaner flotation, the pH regulator B, the depressant B, the collector B, and the frother B are added in this order to the (j-1)^{th}-stage second cleaner flotation concentrate slurry.

These reagents are added at an interval of 2 to 5 minutes, preferably 3 to 4 minutes. The interval is calculated by the following formula: t=t₁-t₂, where t is the interval, t₁ is the time of starting the addition of a next reagent, and t₂ is the time of completing the addition of a preceding reagent.

The concentration of the (j-1)^{th}-stage second cleaner flotation concentrate slurry may be 35 to 55 wt%, preferably 40 to 50 wt%, and more preferably 40 to 45 wt%.

The j^{th}-stage second cleaner flotation may be carried out at a temperature of 35 to 65 °C, preferably 40 to 60 °C, and more preferably 50 to 55 °C.

Preferably, I is 3, meaning that three-stage second cleaner flotation is carried out.

In the 2^{nd}-stage second cleaner flotation, the pH regulator B may be in an amount of 0.10 to 0.30 kg/T, preferably 0.15 to 0.25 kg/T, and more preferably 0.20 to 0.23 kg/T, based on the weight of the mixed rare earth ore.

In the 2^{nd}-stage second cleaner flotation, the depressant B may be in an amount of 0.15 to 0.35 kg/T, preferably 0.20 to 0.30 kg/T, based on the weight of the mixed rare earth ore. In some embodiments, the depressant B is in an amount of 0.22 to 0.23 kg/T.

In the 2^{nd}-stage second cleaner flotation, the collector B may be in an amount of 0.10 to 0.25 kg/T, preferably 0.15 to 0.20 kg/T, and more preferably 0.17 to 0.18 kg/T, based on the weight of the mixed rare earth ore.

In the 2^{nd}-stage second cleaner flotation, the frother B may be in an amount of 0.02 to 0.06 kg/T, preferably 0.03 to 0.05 kg/T, based on the weight of the mixed rare earth ore. In some embodiments, the frother B is in an amount of 0.04 to 0.045 kg/T.

In the 3^{rd}-stage second cleaner flotation, the pH regulator B may be in an amount of 0.05 to 0.30 kg/T, preferably 0.08 to 0.25 kg/T, based on the weight of the mixed rare earth ore. In some embodiments, the pH regulator B is in an amount of 0.20 to 0.23 kg/T.

In the 3^{rd}-stage second cleaner flotation, the depressant B may be in an amount of 0.10 to 0.35 kg/T, preferably 0.11 to 0.30 kg/T, based on the weight of the mixed rare earth ore. In some embodiments, the depressant B is in an amount of 0.25 to 0.28 kg/T.

In the 3^{rd}-stage second cleaner flotation, the collector B may be in an amount of 0.07 to 0.25 kg/T, preferably 0.085 to 0.20 kg/T, based on the weight of the mixed rare earth ore. In some embodiments, the collector B is in an amount of 0.15 to 0.17 kg/T.

In 3^{rd}-stage second cleaner flotation, the frother B may be in an amount of 0.01 to 0.06 kg/T, preferably 0.02 to 0.05 kg/T, based on the weight of the mixed rare earth ore. In some embodiments, the frother B is in an amount of 0.04 to 0.05 kg/T.

In some embodiments, the method further comprises combining the first flotation concentrate and the second flotation concentrate to produce a rare earth concentrate.

The rare earth concentrate has a rare earth grade of greater than or equal to 30 wt%, preferably greater than or equal to 33 wt%, and more preferably greater than or equal to 36 wt%. The rare earth concentrate may have a rare earth grade of less than or equal to 40 wt%, preferably less than or equal to 38 wt%.

The rare earth recovery rate may be greater than or equal to 70 wt%, preferably greater than or equal to 74 wt%, and more preferably greater than or equal to 79 wt%. The rare earth recovery rate may be less than or equal to 85 wt%. In some embodiments, the rare earth recovery rate is less than or equal to 80 wt%.

### Crushing and Grinding of Mixed Rare Earth Ore

The present disclosure involves crushing mixed rare earth ore to produced crushed ore, and grinding the crushed ore to produce ground mixed rare earth ore.

The crushed ore has a particle size of less than or equal to 5.0 mm, preferably less than or equal to 2.0 mm.

A jaw crusher may be employed to crush mixed rare earth ore to a particle size of less than or equal to 20 mm, preferably less than or equal to 10 mm. A double-roller crusher is then employed for secondary crushing, and a sieve machine is employed for screening, producing crushed ore.

The crushed ore for grinding may have a concentration of 50 to 75 wt%, preferably 60 to 70 wt%, and more preferably 60 to 65 wt%.

The following is a description of testing methods involved in examples given below:
The liberation degree of carbocernaite was tested by an Automated Mineral Identification and Characterization System (AMICS).

The liberation degree of parisite was tested by an Automated Mineral Identification and Characterization System (AMICS).
The REO grade was tested by the method specified in GB/T 18114.1-2010.

The rare earth recovery rate was calculated by this formula: [(REO grade of rare earth concentrate × yield of rare earth concentrate)/REO grade of mixed rare earth ore] × 100%.

The materials employed in the examples are as follows:
The pH regulator was sodium carbonate.

The depressant was a mixture of water glass (sodium silicate with a modulus of 2.4-2.6), sodium hexametaphosphate, and starch in a mass ratio of 6:3:1.

The collector was a mixture of octyl hydroxamic acid and pesticide emulsifier 601 in a mass ratio of 9:1.

The frother was methyl isobutyl carbinol (MIBC).

### Example 1

Crush mixed rare earth ore to particles having a particle size of 10 mm or less using a jaw crusher; and subject the particles to secondary crushing using a double-roller crusher, and screen the particles using a sieve machine to produce crushed ore having a particle size of 2.0 mm or less. The mixed rare earth ore consisted of carbocernaite, parisite, and a gangue. The mass ratio of carbocernaite to parisite was 4.6:3.7. The gangue included calcite, mica, feldspar, and apatite. The mixed rare earth ore had a REO grade of 3.69 wt% and contained calcite in a content of 42.16 wt%.

Grind the crushed ore using a ball mill, followed by classification and overflow collection, to produce ground mixed rare earth ore (consisting of particles of 86.39 wt% of which had a particle size of 0.074 mm or less). The crushed ore for grinding had a concentration of 62 wt%. In the ground mixed rare earth ore, carbocernaite had a liberation degree of 83.66%, and parisite had a liberation degree of 24.18%.

Subject the ground mixed rare earth ore to rougher magnetic separation to produce a rougher magnetic concentrate and a rougher magnetic tailing. Subject the rougher magnetic tailing to scavenger magnetic separation to produce a scavenger magnetic concentrate and a magnetic tailing. Combine the rougher magnetic concentrate and the scavenger magnetic concentrate to produce a magnetic concentrate. The rougher magnetic separation was performed at a field intensity of 1.2 T and a pulse frequency of 15 Hz and used the ground mixed rare earth ore having a concentration of 20 wt%. The scavenger magnetic separation was performed at a field intensity of 1.7 T and a pulse frequency of 18 Hz and used the rougher magnetic tailing having a concentration of 20 wt%.

Form a magnetic concentrate slurry having a concentration of 55 wt% from the magnetic concentrate. Subject the magnetic concentrate slurry to first rougher flotation by adding thereto at 60 °C the pH regulator, the depressant, the collector, and the frother in this order at an interval of 3 minutes to produce a first rougher flotation concentrate and a first flotation tailing. The amount of the pH regulator was 1.4 kg/t, the amount of the depressant was 2.2 kg/t, the amount of the collector was 1.2 kg/t, and the amount of the frother was 0.18 kg/t, based on the weight of the mixed rare earth ore.

Form a first rougher flotation concentrate slurry having a concentration of 58 wt% from the first rougher flotation concentrate. Subject the first rougher flotation concentrate slurry to 1^{st}-stage first cleaner flotation by adding thereto at 50 °C and the pH regulator, the depressant, the collector, and the frother in this order at an interval of 3 minutes to produce a 1^{st}-stage first cleaner flotation concentrate and a 1^{st}-stage first cleaner flotation tailing. Return the 1^{st}-stage first cleaner flotation tailing as a feed material to the first rougher flotation. The amount of the pH regulator was 0.42 kg/t, the amount of the depressant was 0.66 kg/t, the amount of the collector was 0.36 kg/t, and the amount of the frother was 0.054 kg/t, based on the weight of the mixed rare earth ore.

Form a 1^{st}-stage first cleaner flotation concentrate slurry having a concentration of 50 wt% from the 1^{st}-stage first cleaner flotation concentrate. Subject the 1^{st}-stage first cleaner flotation concentrate slurry to 2^{nd}-stage first cleaner flotation by adding thereto at 50 °C the pH regulator, the depressant, the collector, and the frother in this order at an interval of 3 minutes to produce a 2^{nd}-stage first cleaner flotation concentrate and a 2^{nd}-stage first cleaner flotation tailing. Return the 2^{nd}-stage first cleaner flotation tailing as a feed material to the 1^{st}-stage first cleaner flotation. The amount of the pH regulator was 0.14 kg/t, the amount of the depressant was 0.22 kg/t, the amount of the collector was 0.12 kg/t, and the amount of the frother was 0.018 kg/t, based on the weight of the mixed rare earth ore.

Form a 2^{nd}-stage first cleaner flotation concentrate slurry having a concentration of 48 wt% from the 2^{nd}-stage first cleaner flotation concentrate. Subject the 2^{nd}-stage first cleaner flotation concentrate slurry to 3^{rd}-stage first cleaner flotation by adding thereto at 55 °C the pH regulator, the depressant, the collector, and the frother in this order at an interval of 3 minutes to produce a 3^{rd}-stage first cleaner flotation concentrate and a 3^{rd}-stage first cleaner flotation tailing. Return the 3^{rd}-stage first cleaner flotation tailing as a feed material to the 2^{nd}-stage first cleaner flotation. Designate the 3^{rd}-stage first cleaner flotation concentrate as the first flotation concentrate. The amount of the pH regulator was 0.14 kg/t, the amount of the depressant was 0.22 kg/t, the amount of the collector was 0.12 kg/t, and the amount of the frother was 0.018 kg/t, based on the weight of the mixed rare earth ore.

Grind the first flotation tailing using IsaMill, followed by classification and overflow collection, to produce a ground first flotation tailing (consisting of particles 93.15 wt% of which had a particle size of 0.03 mm or less). The first flotation tailing for grinding had a concentration of 60 wt%. In the ground first flotation tailing, parisite had a liberation degree of 82%.

Form a ground first flotation tailing slurry having a concentration of 45 wt% from the ground first flotation tailing. Subject the ground first flotation tailing slurry to second rougher flotation by adding thereto at 60 °C the pH regulator, the depressant, the collector, and the frother in this order at an interval of 3 minutes to produce a second rougher flotation concentrate and a second flotation tailing. The amount of the pH regulator was 0.8 kg/t, the amount of the depressant was 1.1 kg/t, the amount of the collector was 0.85 kg/t, and the amount of the frother was 0.2 kg/t, based on the weight of the mixed rare earth ore.

Form a second rougher flotation concentrate slurry having a concentration of 45 wt% from the second rougher flotation concentrate. Subject the second rougher flotation concentrate slurry to 1^{st}-stage second cleaner flotation by adding thereto at 50 °C the pH regulator, the depressant, the collector, and the frother in this order at an interval of 3 minutes to produce a 1^{st}-stage second cleaner flotation concentrate and 1^{st}-stage second cleaner flotation tailing. Return the 1^{st}-stage second cleaner flotation tailing as a feed material to the second rougher flotation. The amount of the pH regulator was 0.32 kg/t, the amount of the depressant was 0.44 kg/t, the amount of the collector was 0.34 kg/t, and the amount of the frother was 0.08 kg/t, based on the weight of the mixed rare earth ore.

Form a 1^{st}-stage second cleaner flotation concentrate slurry having a concentration of 42 wt% from the 1^{st}-stage second cleaner flotation concentrate. Subject the 1^{st}-stage second cleaner flotation concentrate slurry to 2^{nd}-stage second cleaner flotation by adding thereto at 50 °C the pH regulator, the depressant, the collector, and the frother in this order at an interval of 3 minutes to produce a 2^{nd}-stage second cleaner flotation concentrate and a 2^{nd}-stage second cleaner flotation tailing. Return the 2^{nd}-stage second cleaner flotation tailing as a feed material to the 1^{st}-stage second cleaner flotation. The amount of the pH regulator was 0.16 kg/t, the amount of the depressant was 0.22 kg/t, the amount of the collector was 0.17 kg/t, and the amount of the frother was 0.04 kg/t, based on the weight of the mixed rare earth ore.

Form a 2^{nd}-stage second cleaner flotation concentrate slurry having a concentration of 40 wt% from the 2^{nd}-stage second cleaner flotation concentrate. Subject the 2^{nd}-stage second cleaner flotation concentrate slurry to 3^{rd}-stage second cleaner flotation by adding thereto at 50 °C the pH regulator, the depressant, the collector, and the frother in this order at an interval of 3 minutes to produce a 3^{rd}-stage second cleaner flotation concentrate and a 3^{rd}-stage second cleaner flotation tailing. Return the 3^{rd}-stage second cleaner flotation tailing as a feed material to the 2^{nd}-stage second cleaner flotation. Designate the 3^{rd}-stage second cleaner flotation concentrate as the second flotation concentrate. The amount of the pH regulator was 0.08 kg/t, the amount of the depressant was 0.11 kg/t, the amount of the collector was 0.085 kg/t, and the amount of the frother was 0.02 kg/t, based on the weight of the mixed rare earth ore.

Combine the first flotation concentrate and the second flotation concentrate to produce a rare earth concentrate. Combine the magnetic tailing and the second flotation tailing to produce a tailing.

The rare earth concentrate had a REO grade of 36.55 wt%, and the rare earth recovery rate was 74.28 wt%.

### Example 2

Crush mixed rare earth ore to particles having a particle size of 10 mm or less using a jaw crusher; and subject the particles to secondary crushing using a double-roller crusher, and screen the particles using a sieve machine to produce crushed ore having a particle size of 2.0 mm or less. The mixed rare earth ore consisted of carbocernaite, parisite, and a gangue. The mass ratio of carbocernaite to parisite was 5.5:4.5. The gangue included calcite, mica, feldspar, and apatite. The mixed rare earth ore had a REO grade of 4.14 wt% and contained calcite in a content of 45.88 wt%.

Grind the crushed ore using a ball mill, followed by classification and overflow collection, to produce ground mixed rare earth ore (consisting of particles of 89.56 wt% of which had a particle size of 0.074 mm or less). The crushed ore for grinding had a concentration of 65 wt%. In the ground mixed rare earth ore, carbocernaite had a liberation degree of 87.52%, and parisite had a liberation degree of 27.15%.

Subject the ground mixed rare earth ore to rougher magnetic separation to produce a rougher magnetic concentrate and a rougher magnetic tailing. Subject the rougher magnetic tailing to scavenger magnetic separation to produce a scavenger magnetic concentrate and a magnetic tailing. Combine the rougher magnetic concentrate and the scavenger magnetic concentrate to produce a magnetic concentrate. The rougher magnetic separation was performed at a field intensity of 1.4 T and a pulse frequency of 13 Hz and used the ground mixed rare earth having a concentration of 20 wt%. The scavenger magnetic separation was performed at a field intensity of 1.8 T and a pulse frequency of 15 Hz and used the rougher magnetic tailing having a concentration of 20 wt%.

Form a magnetic concentrate slurry having a concentration of 55 wt% from the magnetic concentrate. Subject the magnetic concentrate slurry to first rougher flotation by adding thereto at 60 °C the pH regulator, the depressant, the collector, and the frother in this order at an interval of 3 minutes to produce a first rougher flotation concentrate and a first flotation tailing. The amount of the pH regulator was 1.4 kg/t, the amount of the depressant was 2.2 kg/t, the amount of the collector was 1.2 kg/t, and the amount of the frother was 0.18 kg/t, based on the weight of the mixed rare earth ore.

Form a first rougher flotation concentrate slurry having a concentration of 55 wt% from the first rougher flotation concentrate. Subject the first rougher flotation concentrate slurry to 1^{st}-stage first cleaner flotation by adding thereto at 55 °C and the pH regulator, the depressant, the collector, and the frother in this order at an interval of 3 minutes to produce a 1^{st}-stage first cleaner flotation concentrate and a 1^{st}-stage first cleaner flotation tailing. Return the 1^{st}-stage first cleaner flotation tailing as a feed material to the first rougher flotation. The amount of the pH regulator was 0.42 kg/t, the amount of the depressant was 0.66 kg/t, the amount of the collector was 0.36 kg/t, and the amount of the frother was 0.054 kg/t, based on the weight of the mixed rare earth ore.

Form a 1^{st}-stage first cleaner flotation concentrate slurry having a concentration of 48 wt% from the 1^{st}-stage first cleaner flotation concentrate. Subject the 1^{st}-stage first cleaner flotation concentrate slurry to 2^{nd}-stage first cleaner flotation by adding thereto at 50 °C the pH regulator, the depressant, the collector, and the frother in this order at an interval of 3 minutes to produce a 2^{nd}-stage first cleaner flotation concentrate and a 2^{nd}-stage first cleaner flotation tailing. Return the 2^{nd}-stage first cleaner flotation tailing as a feed material to the 1^{st}-stage first cleaner flotation. The amount of the pH regulator was 0.14 kg/t, the amount of the depressant was 0.22 kg/t, the amount of the collector was 0.12 kg/t, and the amount of the frother was 0.018 kg/t, based on the weight of the mixed rare earth ore.

Form a 2^{nd}-stage first cleaner flotation concentrate slurry having a concentration of 45 wt% from the 2^{nd}-stage first cleaner flotation concentrate. Subject the 2^{nd}-stage first cleaner flotation concentrate slurry to 3^{rd}-stage first cleaner flotation by adding thereto at 50 °C the pH regulator, the depressant, the collector, and the frother in this order at an interval of 3 minutes to produce a 3^{rd}-stage first cleaner flotation concentrate and a 3^{rd}-stage first cleaner flotation tailing. Return the 3^{rd}-stage first cleaner flotation tailing as a feed material to the 2^{nd}-stage first cleaner flotation. Designate the 3^{rd}-stage first cleaner flotation concentrate as the first flotation concentrate. The amount of the pH regulator was 0.14 kg/t, the amount of the depressant was 0.22 kg/t, the amount of the collector was 0.12 kg/t, and the amount of the frother was 0.018 kg/t, based on the weight of the mixed rare earth ore.

Grind the first flotation tailing using IsaMill, followed by classification and overflow collection, to produce a ground first flotation tailing (consisting of particles 90.44 wt% of which had a particle size of 0.03 mm or less). The first flotation tailing for grinding had a concentration of 55 wt%. In the ground first flotation tailing, parisite had a liberation degree of 78%.

Form a ground first flotation tailing slurry having a concentration of 50 wt% from the ground first flotation tailing. Subject the ground first flotation tailing slurry to second rougher flotation by adding thereto at 65 °C the pH regulator, the depressant, the collector, and the frother in this order at an interval of 3 minutes to produce a second rougher flotation concentrate and a second flotation tailing. The amount of the pH regulator was 1.1 kg/t, the amount of the depressant was 1.3 kg/t, the amount of the collector was 0.75 kg/t, and the amount of the frother was 0.25 kg/t, based on the weight of the mixed rare earth ore.

Form a second rougher flotation concentrate slurry having a concentration of 48 wt% from the second rougher flotation concentrate. Subject the second rougher flotation concentrate slurry to 1^{st}-stage second cleaner flotation by adding thereto at 55 °C the pH regulator, the depressant, the collector, and the frother in this order at an interval of 3 minutes to produce a 1^{st}-stage second cleaner flotation concentrate and 1^{st}-stage second cleaner flotation tailing. Return the 1^{st}-stage second cleaner flotation tailing as a feed material to the second rougher flotation. The amount of the pH regulator was 0.33 kg/t, the amount of the depressant was 0.39 kg/t, the amount of the collector was 0.225 kg/t, and the amount of the frother was 0.075 kg/t, based on the weight of the mixed rare earth ore.

Form a 1^{st}-stage second cleaner flotation concentrate slurry having a concentration of 45 wt% from the 1^{st}-stage second cleaner flotation concentrate. Subject the 1^{st}-stage second cleaner flotation concentrate slurry to 2^{nd}-stage second cleaner flotation by adding thereto at 52 °C the pH regulator, the depressant, the collector, and the frother in this order at an interval of 3 minutes to produce a 2^{nd}-stage second cleaner flotation concentrate and a 2^{nd}-stage second cleaner flotation tailing. Return the 2^{nd}-stage second cleaner flotation tailing as a feed material to the 1^{st}-stage second cleaner flotation. The amount of the pH regulator was 0.22 kg/t, the amount of the depressant was 0.26 kg/t, the amount of the collector was 0.15 kg/t, and the amount of the frother was 0.05 kg/t, based on the weight of the mixed rare earth ore.

Form a 2^{nd}-stage second cleaner flotation concentrate slurry having a concentration of 42 wt% from the 2^{nd}-stage second cleaner flotation concentrate. Subject the 2^{nd}-stage second cleaner flotation concentrate slurry to 3^{rd}-stage second cleaner flotation by adding thereto at 50 °C the pH regulator, the depressant, the collector, and the frother in this order at an interval of 3 minutes to produce a 3^{rd}-stage second cleaner flotation concentrate and a 3^{rd}-stage second cleaner flotation tailing. Return the 3^{rd}-stage second cleaner flotation tailing as a feed material to the 2^{nd}-stage second cleaner flotation. Designate the 3^{rd}-stage second cleaner flotation concentrate as the second flotation concentrate. The amount of the pH regulator was 0.22 kg/t, the amount of the depressant was 0.26 kg/t, the amount of the collector was 0.15 kg/t, and the amount of the frother was 0.05 kg/t, based on the weight of the mixed rare earth ore.

Combine the first flotation concentrate and the second flotation concentrate to produce a rare earth concentrate. Combine the magnetic tailing and the second flotation tailing to produce a tailing.

The rare earth concentrate had a REO grade of 33.82 wt%, and the rare earth recovery rate was 79.51 wt%.

The present disclosure is not limited to the embodiments described above. Any variation, improvement, and replacement which do not depart from the essence of the present disclosure and which those skilled in the art are able to think of fall within the scope of the present disclosure.

## Claims

1. A beneficiation method for mixed rare earth ore, comprising:
(1) subjecting ground mixed rare earth ore to magnetic separation to produce a magnetic concentrate and a magnetic tailing, wherein the mixed rare earth ore contains carbocernaite and parisite;
(2) subjecting the magnetic concentrate to first flotation in the presence of a pH regulator A, a depressant A, a collector A, and a frother A to produce a first flotation concentrate and a first flotation tailing,
wherein the depressant A comprises water glass, a phosphate, and starch in a mass ratio of (4-8):(1-5):(0.5-3), the collector A comprises a C5-C10 hydroxamic acid and a styrylphenol polyoxyethylene ether in a mass ratio of (7-11):(0.5-3), and the frother A is a fatty alcohol frother;
(3) grinding the first flotation tailing to produce a ground first flotation tailing; and
(4) subjecting the ground first flotation tailing to second flotation in the presence of a pH regulator B, a depressant B, a collector B, and a frother B to produce a second flotation concentrate and a second flotation tailing,
wherein the depressant B comprises water glass, a phosphate, and starch in a mass ratio of (4-8):(1-5):(0.5-3), the collector B comprises a C5-C10 hydroxamic acid and a styrylphenol polyoxyethylene ether in a mass ratio of (7-11):(0.5-3), and the frother B is a fatty alcohol frother.

2. The beneficiation method according to claim 1, wherein step (1) comprises:
subjecting ground mixed rare earth ore to rougher magnetic separation to produce a rougher magnetic concentrate and a rougher magnetic tailing, wherein the rougher magnetic separation is performed at a field intensity of 1.1-1.5 T and a pulse frequency of 12-16 Hz and uses the ground mixed rare earth ore having a concentration of 10-30 wt%;
subjecting the rougher magnetic tailing to scavenger magnetic separation to produce a scavenger magnetic concentrate and a magnetic tailing, wherein the scavenger magnetic separation is performed at a field intensity of 1.6-2.0 T and a pulse frequency of 13-20 Hz and uses the rougher magnetic tailing having a concentration of 10-30 wt%; and
combining the rougher magnetic concentrate and the scavenger magnetic concentrate to produce a magnetic concentrate,
wherein the ground mixed rare earth ore consists of particles 75-100 wt% of which have a particle size of 0.074 mm or less.

3. The beneficiation method according to claim 1, wherein the water glass has a modulus of 2-3, the phosphate is one or more selected from the group consisting of sodium hexametaphosphate and trisodium phosphate, the hydroxamic acid is a C7-9 hydroxamic acid, the styrylphenol polyoxyethylene ether is one or more selected from the group consisting of pesticide emulsifier 601, pesticide emulsifier 602, pesticide emulsifier 603, and pesticide emulsifier 604, the fatty alcohol frother is a C4-C10 aliphatic monohydric alcohol, the pH regulator A is a carbonate, and the pH regulator B is a carbonate.

4. The beneficiation method according to claim 1, wherein step (2) comprises:
forming a magnetic concentrate slurry having a concentration of 45-65 wt% from the magnetic concentrate; subjecting the magnetic concentrate slurry to first rougher flotation by adding thereto at 50-70 °C a pH regulator A, a depressant A, a collector A, and a frother A to produce a first rougher flotation concentrate and a first flotation tailing, wherein the pH regulator A is in an amount of 1.0-2.0 kg/T, the depressant A is in an amount of 1.5-2.5 kg/T, the collector A is in an amount of 0.9-1.5 kg/T, and the frother A is in an amount of 0.1-0.3 kg/T, based on the weight of the mixed rare earth ore; and
subjecting the first rougher flotation concentrate to N-stage first cleaner flotation to produce a first flotation concentrate, wherein N is an integer greater than or equal to 2,
wherein 1^{st}-stage first cleaner flotation comprises: forming a first rougher flotation concentrate slurry from the first rougher flotation concentrate; subjecting the first rougher flotation concentrate slurry to 1^{st}-stage first cleaner flotation by adding thereto a pH regulator A, a depressant A, a collector A, and a frother A to produce a 1^{st}-stage first cleaner flotation concentrate and a 1^{st}-stage first cleaner flotation tailing; and returning the 1^{st}-stage first cleaner flotation tailing as a feed material to the first rougher flotation, wherein the pH regulator A is in an amount of 0.2-0.6 kg/T, the depressant A is in an amount of 0.4-0.9 kg/T, the collector A is in an amount of 0.1-0.5 kg/T, and the frother A is in an amount of 0.01-0.2 kg/T, based on the weight of the mixed rare earth ore, and
wherein each of 2^{nd}-stage first cleaner flotation to N^{th}-stage first cleaner flotation comprises: forming a (m-1)^{th}-stage first cleaner flotation concentrate slurry from a (m-1)^{th}-stage first cleaner flotation concentrate; subjecting the (m-1)^{th}-stage first cleaner flotation concentrate slurry to m^{th}-stage first cleaner flotation by adding thereto a pH regulator A, a depressant A, a collector A, and a frother A to produce a m^{th}-stage first cleaner flotation concentrate and a m^{th}-stage first cleaner flotation tailing; and returning the m^{th}-stage first cleaner flotation tailing as a feed material to the (m-1)^{th}- stage first cleaner flotation, wherein the pH regulator A is in an amount of 0.05-0.25 kg/T, the depressant A is in an amount of 0.10-0.35 kg/T, the collector A is in an amount of 0.05-0.25 kg/T, and the frother A is in an amount of 0.005-0.035 kg/T, based on the weight of the mixed rare earth ore, m is an integer greater than or equal to 2 and less than or equal to N, and the N^{th}-stage first cleaner flotation concentrate is the first flotation concentrate.

5. The beneficiation method according to claim 4, wherein in step (2), the pH regulator A, the depressant A, the collector A, and the frother A are added in this order at an interval of 2-5 minutes,
wherein the interval is calculated by the following formula: $t = {t}_{1} - {t}_{2}$ where t is the interval, t₁ is the time of starting the addition of a next reagent, and t₂ is the time of completing the addition of a preceding reagent.

6. The beneficiation method according to claim 1, wherein in step (3), the first flotation tailing for grinding has a concentration of 50-65 wt%, and the ground first flotation tailing consists of particles 85-100 wt% of which have a particle size of 0.03 mm or less.

7. The beneficiation method according to claim 1, wherein step (4) comprises:
forming a first flotation tailing slurry having a concentration of 40-65 wt% from the ground first flotation tailing; subjecting the first flotation tailing slurry to second rougher flotation by adding thereto at 50-70 °C a pH regulator B, a depressant B, a collector B, and a frother B to produce a second rougher flotation concentrate and a second flotation tailing, wherein the pH regulator B is in an amount of 0.6-1.3 kg/T, the depressant B is in an amount of 0.8-1.6 kg/T, the collector B is in an amount of 0.5-1.1 kg/T, and the frother B is in an amount of 0.1-0.5 kg/T, based on the weight of the mixed rare earth ore; and
subjecting the second rougher flotation concentrate to I-stage second cleaner flotation to produce a second flotation concentrate, wherein I is an integer greater than or equal to 2,
wherein 1^{st}-stage second cleaner flotation comprises:
forming a second rougher flotation concentrate slurry from the second rougher flotation concentrate; subjecting the second rougher flotation concentrate slurry to 1^{st}-stage second cleaner flotation by adding thereto a pH regulator B, a depressant B, a collector B, and a frother B to produce a 1^{st}-stage second cleaner flotation concentrate and a 1^{st}-stage second cleaner flotation tailing; and returning the 1^{st}-stage second cleaner flotation tailing as a feed material to the second rougher flotation, wherein the pH regulator B is in an amount of 0.2-0.5 kg/T, the depressant B is in an amount of 0.2-0.6 kg/T, the collector B is in an amount of 0.1-0.5 kg/T, and the frother B is in an amount of 0.01-0.15 kg/T, based on the weight of the mixed rare earth ore,
wherein each of 2^{nd}-stage second cleaner flotation to I^{th}-stage second cleaner flotation comprises:
forming a (j-1)^{th}-stage second cleaner flotation concentrate slurry from a (j-1)^{th}-stage second cleaner flotation concentrate; subjecting the (j-1)^{th}-stage second cleaner flotation concentrate slurry to j^{th}-stage second cleaner flotation by adding thereto a pH regulator B, a depressant B, a collector B, and a frother B to produce a j^{th}-stage second cleaner flotation concentrate and a j^{th}-stage second cleaner flotation tailing; and returning the j^{th}-stage second cleaner flotation tailing as a feed material to the (j-1)^{th}-stage second cleaner flotation, wherein the pH regulator B is in an amount of 0.05-0.30 kg/T, the depressant B is in an amount of 0.08-0.35 kg/T, the collector B is in an amount of 0.05-0.25 kg/T, and the frother B is in an amount of 0.005-0.07 kg/T, based on the weight of the mixed rare earth ore, j is an integer greater than or equal to 2 and less than or equal to I, and the I^{th}-stage second cleaner flotation concentrate is the second flotation concentrate.

8. The beneficiation method according to claim 7, wherein in step (4), the pH regulator B, the depressant B, the collector B, and the frother B are added in this order at an interval of 2-5 minutes,
wherein the interval is calculated by the following formula: $t = {t}_{1} - {t}_{2}$ where t is the interval, t₁ is the time of starting the addition of a next reagent, and t₂ is the time of completing the addition of a preceding reagent.

9. The beneficiation method according to claim 1, comprising:
combining the first flotation concentrate and the second flotation concentrate to produce a rare earth concentrate.

10. The beneficiation method according to claim 1, further comprising:
crushing the mixed rare earth ore to produce crushed ore; and grinding the crushed ore to produce ground mixed rare earth ore,
wherein the mixed rare earth ore contains carbocernaite and parisite in a mass ratio of (3-6.5):(2-5.5), and further contains at least one of calcite, mica, feldspar, and apatite.
